

T. M. OWEN,

APPARATUS FOR THE CONCENTRATION OF ORES.  
APPLICATION FILED MAY 2, 1914.

1,155,836.

Patented Oct. 5, 1915.

2 SHEETS—SHEET 1.

Fig. 1.



*Witnesses:*

Harry P. Lewis  
Kenneth D. Widdemer

*Inventor:*

Thomas Mackellar Owen

by Henry B. Williams  
Attorney.

T. M. OWEN,  
APPARATUS FOR THE CONCENTRATION OF ORES,  
APPLICATION FILED MAY 2, 1914.

1,155,836.

Patented Oct. 5, 1915.

2 SHEETS—SHEET 2.



# UNITED STATES PATENT OFFICE.

THOMAS MACKELLAR OWEN, OF BROKEN HILL, NEW SOUTH WALES, AUSTRALIA,  
ASSIGNOR TO MINERALS SEPARATION AMERICAN SYNDICATE (1913) LIMITED, OF  
LONDON, ENGLAND.

## APPARATUS FOR THE CONCENTRATION OF ORES.

1,155,836.

Specification of Letters Patent.

Patented Oct. 5, 1915.

Application filed May 2, 1914. Serial No. 835,811.

*To all whom it may concern:*

Be it known that I, THOMAS MACKELLAR OWEN, a subject of the King of England, residing at Broken Hill, New South Wales, 5 Australia, have invented certain new and useful Improvements in Apparatus for the Concentration of Ores, of which the following is a specification.

This invention is for improvements in or 10 relating to apparatus for ore concentration.

The apparatus is intended for carrying out the agitation-froth process as described for example in the previous United States 15 patents of Sulman, Picard and Ballot, No. 835,120, issued November 6, 1906, of Sulman, Greenway and Higgins, No. 962,678, issued June 28, 1910, and of Greenway and Lavers, No. 1,064,723, issued June 17, 1913, and is particularly well adapted for dif- 20 ferential flotation, as described, for example, in United States patent to Nutter and Lavers, No. 1,067,485, issued July 15, 1913.

Hitherto it has been common practice to introduce the ore pulp with the agents necessary for froth formation into an agitation vessel where the pulp was subjected to violent agitation accompanied by the beating in of the supernatant air, after which the pulp (containing a potential froth) was dis- 25 charged into a separate spitzkasten in which the froth floated and was separated.

My invention consists of an ore concentration apparatus in which the air or other gas is introduced into the lower part of the 30 apparatus and in which the agitation of the pulp and minute division of the air (or air emulsification) takes place in such lower part of the apparatus, and in which the agitated pulp and air emulsion are allowed to 35 pass upwardly and means are interposed in their upward movement for producing a condition of comparative quiescence at the 40 upper part of the apparatus so that the froth may rise to the surface of the pulp and float off from or be removed from such 45 surface.

My invention includes an apparatus in which the agitation and aeration of the pulp and the formation and flotation of the froth 50 can take place in one vessel, so that the mineral-bearing froth can be produced continuously and removed from the surface of the pulp as soon as it is formed. In such apparatus, the pulp in the upper part of the ves-

sel is subjected to a continuous stream of minute air bubbles, and this stream of minute air bubbles may be regulated as desired. 55

The accompanying drawings illustrate apparatus embodying my invention. I will now particularly describe such apparatus 60 and will thereafter point out my invention in claims.

Figure 1 is a vertical central section of one form of apparatus embodying my invention. Fig. 2 is a vertical central section of another form of such apparatus. Fig. 3 is a horizontal section taken on the line 3—3 of Fig. 2.

Referring first to Fig. 1 a vertical glass cylinder A with open top has a neck at the 70 bottom with a central orifice B provided with a regulating valve C. At the bottom of the vessel is a paddle or propeller agitator D with inclined blades. The paddle is carried on a vertical spindle which is rotated 75 at a high speed in such a direction as to throw the liquid contents upward. Immediately above the top of the paddle a ring I carrying four vertical baffles E is fitted into the cylinder. These baffles terminate a 80 substantial distance below the surface of the liquid in the cylinder. The normal level of still liquid is indicated by the broken line X.

At the top of the apparatus an overflow launder Y is provided which performs the 85 usual function of receiving and carrying off the floating concentrate. In operation the air or other gas is admitted to the apparatus through the orifice B at the bottom, the amount being regulated and controlled 90 by adjustment of the valve C, and the air or other gas is delivered toward the agitator D. Three zones of different character are produced in the apparatus; F the "atomizing zone" being the zone of intense agitation 95 and aeration near the bottom of the vessel; G the "baffling zone" where the whirl of the mass is broken up; H the "separating zone" where the liquid mass is sufficiently still to allow of the froth separation taking place. 100

Such an apparatus may be used intermittently or continuously that is to say, the overflow may be continuous or the froth may be periodically removed by introducing sufficient liquid to cause the overflow. It is possible with an apparatus of this sort to treat 105 a given charge of pulp and continuously or intermittently to remove the froth until the

rising froth is white and contains no mineral. Such an apparatus is particularly suitable for carrying out laboratory tests, but may also be used on a large scale for 5 commercial operations.

Referring to Fig. 2, the apparatus here shown comprises a vertical cylindrical vessel J having a conical bottom K and a tapered or conical upper portion L. An inlet conduit M for ore pulp leads into the bottom of this vessel. An inlet conduit N for air also leads into the bottom of the vessel; preferably centrally therein, and a valve O is arranged in this conduit to control the air admission. A rotating agitator D is located near the bottom of the vessel and four vertical baffles E' are located in the vessel above the agitator. At the top of the vessel an overflow launder Q is provided. An outlet conduit T for the depleted tailings is located in the upper conical part of the vessel. The operation is as follows: An ore pulp with a frothing agent (such as eucalyptus oil) is introduced into the vessel J through the pulp inlet M, air is introduced through the air inlet N and may be supplied under pressure, and the flow of air is regulated by the valve O. The ore pulp is violently agitated with the air and flows upward and 30 its turbulence is restrained by the vertical baffles E', so that at the top of the vessel the pulp is comparatively still and the froth forms and overflows into the concentrates launder Q, while the depleted ore pulp flows 35 out of the vessel through the outlet conduit T. The operation is preferably continuous.

Although air is preferably used, obviously any other gas may be employed. The apparatus is well adapted for flotation of all of 40 the mineral content of an ore or for fractional or differential flotation of part of the mineral contents of an ore, and the capacity of regulating the inflow of the supply of air or other gas makes it particularly useful for 45 fractional or differential flotation.

What I claim as my invention and desire to secure by Letters Patent is:—

1. In an apparatus for concentrating ores by gaseous flotation of certain mineral particles in liquid, a single upright vessel open at the top comprising both an agitation and a separation vessel, an inlet conduit for ore pulp at the bottom of the vessel, an outlet conduit for tailings near the top of the 50 vessel, a rotatable agitator in the lower part of the vessel, a conduit for air leading into

the lower part of the vessel, vertically elongated baffles immediately above the agitator terminating at a substantial distance below the surface of the liquid in the vessel for 60 producing a baffling zone above the atomizing zone and a substantially quiescent topmost and separating zone above the baffling zone.

2. In an apparatus for concentrating ores 65 by gaseous flotation of certain mineral particles in liquid, a single upright vessel open at the top comprising both an agitation and a separation vessel, an inlet conduit for ore pulp at the bottom of the vessel, an outlet conduit for tailings near the top of the vessel, a rotatable agitator in the lower part of the vessel, a conduit for air leading into the lower part of the vessel, vertically elongated baffles immediately above the agitator 70 terminating at a substantial distance below the surface of the liquid in the vessel for producing a baffling zone above the atomizing zone and a substantially quiescent topmost and separating zone above the 75 baffling zone, and a concentrates launder arranged at the top of the vessel for continuous removal of froth.

3. In an apparatus for concentrating ores 80 by gaseous flotation of certain mineral particles in liquid, a single upright cylindrically shaped vessel comprising both an agitation and a separation vessel, an inlet conduit for ore pulp at the bottom of the vessel, an outlet conduit for tailings near the top 85 of the vessel, a rotatable agitator in the lower part of the vessel, an air conduit for air leading into the lower part of the vessel, a valve in the air conduit for regulating the amount of air delivered to the agitation 90 zone, four vertically elongated baffles above the agitator terminating at a substantial distance below the surface of the liquid in the vessel for producing a baffling zone above the atomizing zone and a substantially quiescent 95 topmost and separating zone above the baffling zone, and a concentrates launder arranged at the top of the vessel for continuous removal of froth.

In testimony whereof I have signed my 100 name to this specification in the presence of two subscribing witnesses.

THOMAS MACKELLAR OWEN.

Witnesses:

HENRY D. WILLIAMS,  
HARRY C. LEWIS.